

Feb. 13, 1962

C. GUILLAUD

3,021,283

FERROMAGNETIC MATERIALS WITH LOW COEFFICIENT OF TEMPERATURE  
OF THE INITIAL MAGNETIC PERMEABILITY

Filed Jan. 3, 1958

2 Sheets-Sheet 1



Inventor  
**C. GUILLAUD**

By *John M. Calmapple*  
Attorney

Feb. 13, 1962

C. GUILLAUD

3,021,283

FERROMAGNETIC MATERIALS WITH LOW COEFFICIENT OF TEMPERATURE  
OF THE INITIAL MAGNETIC PERMEABILITY

Filed Jan. 3, 1958

2 Sheets-Sheet 2



Inventor

C. GUILLAUD

By *John M. Calmafka*  
Attorney

## 1

3,021,283

## FERROMAGNETIC MATERIALS WITH LOW COEFFICIENT OF TEMPERATURE OF THE INITIAL MAGNETIC PERMEABILITY

Charles Guillaud, Bellevue, France, assignor to Centre National de la Recherche Scientifique, Paris, France, a corporation of France

Filed Jan. 3, 1958, Ser. No. 707,049

Claims priority, application France Jan. 8, 1957

2 Claims. (Cl. 252—62.5)

The invention relates to ferromagnetic materials with low temperature coefficient of the initial permeability, said materials consisting of solid homogeneous solutions of metallic oxides comprising oxides of iron  $Fe_2O_3$  and  $FeO$ , the latter oxide not necessarily being present, of nickel oxide  $NiO$ , zinc oxide  $ZnO$ , aluminum oxide  $Al_2O_3$ , chromium oxide  $Cr_2O_3$ , the two latter oxides may be together or separately.

It is known that these materials are prepared, generally speaking, by subjecting to a heat treatment a pulverulent mixture comprising the above-mentioned oxides previously agglomerated under pressure to the desired form.

The invention also relates to a method of manufacturing said materials.

In order to permit a better understanding of the following, we will first of all define an essential characteristic of the materials concerned.

It is known that the initial magnetic permeability of ferromagnetic materials varies more or less as a function of the temperature. The amplitude of this variation is conveniently expressed by a magnitude known as "coefficient of temperature of the initial magnetic permeability." This coefficient will hereinafter be described by " $\alpha\mu$ ." By this term is meant the difference between the maximum initial ( $-\mu_{\max}$ ) and minimum ( $-\mu_{\min}$ ) magnetic permeabilities marked in a given temperature interval  $t_1$  and  $t_2$  this difference being divided by the product of the initial magnetic permeability ( $-\mu_0$ ) measured at  $0^\circ C$ . and the difference between the limit temperatures of this interval:

$$\alpha\mu = \frac{1}{\mu_0} \frac{\mu_{\max} - \mu_{\min}}{t_2 - t_1}$$

It is also possible to give this coefficient in percent per degrees centigrade (this numerical value then being the centuple of that corresponding to the above formula).

For certain practical applications, the coefficients of temperature of the initial magnetic permeability must be very low and this within a large temperature interval. Thus, materials having the same composition of oxide of nickel and zinc as those which will be specified in the following, but of which the oxides of aluminum and chromium have been replaced by oxide of iron, cannot be used owing to the fact that the amplitude of variation of the initial magnetic permeability is too high.

The object of the present invention is to give the compositions and the methods of manufacture making it possible to obtain materials having low coefficients of temperature of the initial magnetic permeability in temperature intervals which may exceed  $100^\circ C$ , while maintaining their magnetic permeability sufficiently high.

For this purpose a starting mixture of oxides of iron, aluminum, chromium, nickel and zinc is prepared, comprising in molecular percentage: 33% to 50% of iron oxide  $Fe_2O_3$ , 16% to 23% of nickel oxide, 1% to 15% of aluminum or chromium oxide or of the total of these two latter oxides, the remainder being zinc oxide  $ZnO$ . This mixture, after grinding in a ball mill, usually of steel, is agglomerated under pressure in the form desired. The agglomeration thus obtained is then sintered at a temperature between  $1,100^\circ$  and  $1,350^\circ C$ , in an oxidizing atmos-

## 2

sphere for a time usually spread out between 2 and 4 hours, preferably at  $1,250^\circ C$ . in an atmosphere of pure oxygen for 4 hours.

As has been indicated, the percentages of oxide of aluminum  $Al_2O_3$  or oxide of chromium  $Cr_2O_3$  or again of aluminum oxide  $Al_2O_3$  and chromium oxide  $Cr_2O_3$  may vary within certain limits. They must be determined as a function of the molecular content of nickel-oxide  $NiO$  and of the heat treatment, in such a way that in a temperature interval of at least  $50^\circ C$ , situated between  $-40^\circ$  and  $+80^\circ C$ , the value of the coefficient of temperature of the initial magnetic permeability of the material is less than half the value of the same coefficient measured on a material which has been subjected to the same heat treatment and having the same composition, apart from the fact that the whole of the oxides of chromium and aluminum are replaced by an identical molecular percentage of iron oxide  $Fe_2O_3$ .

In the foregoing, it has been assumed for purposes of simplification in expressing the molecular percentages, that the metals were in the starting mixture solely in the form of oxides of iron  $Fe_2O_3$ , oxide of nickel  $NiO$ , oxide of aluminum  $Al_2O_3$ , oxide of chromium  $Cr_2O_3$ , and zinc oxide  $ZnO$ . They could, however, equally well appear in another form, for example, in the form of other oxides or in the form of salts, in which case it would be sufficient to convert the other oxides, metals or salts really present in the above indicated oxides to equality of the number of metallic atoms.

30 In any case, the invention will be better understood by means of the following non-limitative examples and the attached drawings.

FIG. 1 shows the variation, as a function of the temperature, of the initial magnetic permeability of the materials produced in accordance with the invention, prepared from different starting mixtures all comprising 50% mol. for the combination  $(Fe_2O_3—Al_2O_3)$ , 18% mol. of  $NiO$ , the remainder consisting of  $ZnO$ . The various curves represented each correspond to a particular percentage of oxide  $Al_2O_3$ , which percentage varies from 0 to 10% mol. which has been indicated on the corresponding curve. It is possible to observe how the action of the oxide  $Al_2O_3$  is important on the value of  $\alpha\mu$ , in particular with 7% of  $Al_2O_3$  and, consequently, 43% of  $Fe_2O_3$ , a very low  $\alpha\mu$  is obtained.

FIG. 2 relates to materials comprising 50% mol. for the combination  $(Fe_2O_3—Al_2O_3)$ , 20 mol. of  $NiO$ , the remainder consisting of  $ZnO$ . Each curve relates to a particular content of oxide  $Al_2O_3$ , these contents spreading from 0 to 15% mol. of  $Al_2O_3$ . For a content of 10% of  $Al_2O_3$  the value of  $\alpha\mu$  is very low.

In order to plot the curves represented on FIGS. 1 and 2 and to facilitate comparison, the initial magnetic permeability has, in each case, been conventionally reduced to the value 1,000 at  $0^\circ C$ , by multiplying the real value by a suitable numerical coefficient. The initial magnetic permeability at the other temperatures have been multiplied by the same coefficient.

Unless otherwise indicated in the following examples, 60 the ferromagnetic materials have been prepared by mixing together the oxides in the molecular proportions indicated, by grinding in an aqueous medium by means of a steel ball mill for 24 hours, then drying and compressing in the form of a toroid under a pressure of 5 tons/cm.<sup>2</sup>.

## Example 1

An initial mixture is prepared, containing in molecular proportions: 18% of  $NiO$ , 43% of  $Fe_2O_3$ , 7% of  $Al_2O_3$ , the remainder  $ZnO$ . The heat treatment of the stamped product is effected at  $1,250^\circ C$ . in oxygen for 4 hours and the period of cooling is 15 hours. The coefficient of temperature of the initial permeability measured on one

toroid is .05% per degree centigrade in the interval -40 to +80° C. The coefficient of temperature prepared under the same conditions from a starting mixture containing in molecular proportions 50% of  $Fe_2O_3$ , 18% of  $NiO$  and the remainder of  $ZnO$  is 1.2% per degree centigrade in the temperature interval specified hereinabove.

*Example 2*

A mixture is prepared containing in molecular proportions 20% of  $NiO$ , 40% of  $Fe_2O_3$ , 10% of  $Al_2O_3$ , the remainder being of  $ZnO$ . After heat treatment at 1,250° C. for 4 hours in an oxygen atmosphere and cooling for 16 hours, the coefficient of temperature of the initial permeability measured on a toroid is 0.06% per degree centigrade in the interval -40 to +80° C., while this coefficient measured on a toroid obtained from an initial mixture containing 20% of  $NiO$ , 50% of  $Fe_2O_3$ , the remainder  $ZnO$ , and subjected to the same heat treatments as above is 0.9% per degree centigrade in the interval -40 to +80° C.

*Example 3*

Starting with a mixture containing in molecular proportions: 20% of  $NiO$ , 10% of  $Cr_2O_3$ , 40% of  $Fe_2O_3$ , the remainder  $ZnO$ , there is prepared, using the same thermal conditions as those given in Example 1, a material in the form of a toroid on which a coefficient of temperature of 0.2% per degree centigrade is measured in the interval -40 to +80° C. The coefficient of temperature measured on a toroid prepared under the same thermal conditions as hereinabove from a starting mixture of molecular proportions: 20% of  $NiO$ , 50% of  $Fe_2O_3$  and the remainder  $ZnO$ , is 0.9% per degree centigrade in the same temperature interval.

*Example 4*

From a starting mixture containing in molecular proportions: 19% of  $NiO$ , 5% of  $Al_2O_3$ , 5% of  $Cr_2O_3$ , 39.7% of  $Fe_2O_3$ , the remainder being of  $ZnO$ , a material is prepared using the same heat treatments as those given in Example 1. The coefficient of temperature of the initial

permeability of this material in the interval -40 to +80° C. is 0.07% per degree centigrade.

What I claim is:

5 1. A ferromagnetic ceramic material with a temperature coefficient of initial permeability over a temperature range of at least 50° C. between -40° C. and +80° C. less than a nickel-zinc ferrite over the same temperature range, comprising the reaction product formed by compressing a mixture of 33-50 mol. percent  $Fe_2O_3$ , 16 to 10 20 mol. percent  $NiO$ , containing 5 to 15 mol. percent of a mixture of  $Al_2O_3$  and  $Cr_2O_3$  with the  $Cr_2O_3$  being at least 5 mol. percent and the remainder  $ZnO$ , and heating the compressed mixture in an oxygen atmosphere at a temperature between 1100° C. and 1350° C. for from two to 15 four hours.

2. A ferromagnetic ceramic material having a coefficient of temperature of the initial permeability of approximately 0.07% per degree centigrade over a temperature range of -40° C. to +80° C., comprising the reaction product formed by compressing and heat treating in an oxygen atmosphere at 1250° C. for 4 hours, a mixture of 39.7 mol. percent  $Fe_2O_3$ , 19 mol. percent  $NiO$ , 5 mol. percent  $Al_2O_3$ , 5 mol. percent  $Cr_2O_3$  and the remainder  $ZnO$ .

25

References Cited in the file of this patent

UNITED STATES PATENTS

2,565,861 Leverenz et al. ----- Aug. 28, 1951  
2,576,456 Harvey et al. ----- Nov. 27, 1951  
30 2,640,813 Berge ----- June 2, 1953  
2,723,239 Harvey ----- Nov. 8, 1955

35

FOREIGN PATENTS

1,107,654 France ----- Aug. 10, 1955  
35 1,122,258 France ----- May 22, 1956  
1,128,631 France ----- Aug. 27, 1956  
701,364 Great Britain ----- Dec. 23, 1953  
752,659 Great Britain ----- July 11, 1956

40

OTHER REFERENCES

Economos: J. Amer. Ceramics Soc., July 1955,  
page 242.